

1,551,065

Patented Aug. 25, 1925.

# UNITED STATES PATENT OFFICE.

DANIEL VOORHES SNOWGOOSE, OF NEVADA, MISSOURI

PAVING MATERIAL AND METHOD OF MAKING THE SAME.

No Drawing. Application filed October 10, 1922, Serial No. 593,629. Renewed January 22, 1925.

To all whom it may concern:

Be it known that I, DANIEL V. SNOWGOOSE, a citizen of the United States, residing at Nevada, in the county of Vernon and State of Missouri, have invented a new and useful Paving Material and Method of Making the Same, of which the following is a specification.

This invention relates to a new and improved paving material and to a method of making the same. In some portions of the United States and more especially in the State of Missouri can be found large deposits of a material known as asphalt sand 15 rock or asphalt lime rock. Owing to the peculiar greasy nature of the material it has not been possible, heretofore, to utilize it for any useful purpose. Attempts have been made to employ the material in road building but because of the absence of a 20 binder suitable for holding together the rock particles, such attempts have been unsuccessful. It has been well recognized that the material in question would constitute an 25 excellent base for a road building composition but in the absence of a binder experiments have not resulted successfully.

One of the objects of the present invention is to so treat the material that a suitable binder can be mixed therewith and the resultant product used either in brick form for road building or in sheet form, the road thus constructed being able to withstand the heaviest loads, and being unaffected by atmospheric or climatic changes with the result that it will not crack, warp, or become otherwise distorted. A further object is to provide a road material which will cling to the soil on which it is placed whether this 30 soil be of a sandy or other nature.

With the foregoing and other objects in view the invention consists in certain steps in the method hereinafter pointed out and in certain novel combinations of parts 35 pointed out in the following description and claim.

In preparing the composition the asphalt sand rock or asphalt lime rock is first pulverized, after which it is subjected to the 40 action of heat so that lighter oils contained

therein and consisting of gasoline, kerosene and lubricating oils, will be separated from the sand, the residue being in the form of an asphalt or heavy hydrocarbon and sand.

A hard asphalt is prepared by heating 55 heavy black crude oil thereby to evaporate the lighter oils and to leave a residue of asphalt which is neither brittle nor sticky.

Asphalt sand after being treated by heat as herein described is heated in an open 60 vat or other container and the hard asphalt prepared by the treatment of crude oil is added thereto in the proportion of one part hard asphalt to from five to ten parts of asphalt sand, the exact proportions 65 depending upon the hardness of the product called for in the specifications. In practice the greater the proportion of asphalt to asphalt sand the harder will be the resultant material provided the parts 70 are kept within the proportions above mentioned. After the mixture has been heated in the open container and stirred thoroughly it is ready for use. It can be molded into 75 bricks to be laid in the formation of pavements or roads or it can be molded into large blocks to be subsequently melted and put down as a sheet on a roadway. In practice it has been found that the material thus produced will not soften or melt under 80 the action of the sun's rays. Nor will a pavement of this material crack, warp or otherwise become distorted through expansion or contraction.

What is claimed is:

The herein described method of preparing paving material which consists in reducing asphalt rock to a pulverized state, heating the same to remove therefrom the light oils contained therein, and subsequently mixing the treated rock with hard asphalt while subjected to the action of heat, in the proportions of one part of hard asphalt to from five to ten parts of treated 90 pulverized rock.

In testimony that I claim the foregoing as my own, I have hereto affixed my signature.

DANIEL VOORHES SNOWGOOSE.